

(Model.)

R. MORRISON.

SELF LUBRICATING PACKING FOR STEAM ENGINES, PUMPS, &c.

No. 249,385.

Patented Nov. 8, 1881.



Attest

Will MacGrotty  
Thos. Haughton.

Inventor

Robert Morrison  
P. W. R. Singleton  
Atty

# UNITED STATES PATENT OFFICE.

ROBERT MORRISON, OF ST. LOUIS, MISSOURI.

## SELF-LUBRICATING PACKING FOR STEAM-ENGINES, PUMPS, &c.

SPECIFICATION forming part of Letters Patent No. 249,385, dated November 8, 1881.

Application filed August 27, 1881. (Model.)

To all whom it may concern:

Be it known that I, ROBERT MORRISON, of St. Louis city, and State of Missouri, have invented certain Improvements in Self-Lubricating Packing for Steam Engines, Pumps, &c., of which the following is a specification.

This invention relates to improvements in self-lubricating packing for steam-engines, pumps, and blowing engines, and for all purposes where packing is required; and it consists, first, in equal parts of hemp and cotton fiber spun together into rope of such sizes as may be required to effectually pack a rod, piston, &c.; secondly, in making the rope self-lubricating by the use of plumbago, beeswax, and tallow in such quantities as may be most beneficial to secure a perfect and durable combination of lubricating materials, all of which will be hereinafter more particularly described.

20 The drawing represents a rope formed in accordance with this invention.

The rope is made by spinning together into convenient strands equal quantities of hemp and cotton fiber, which are afterward twisted into rope of the size required. Ten pounds of pulverized plumbago are dusted into the fiber of hemp and cotton to one hundred pounds of those materials while being spun into strands. After being spun these strands are saturated with a mixture of beeswax and tallow in the proportion of fifteen pounds of tallow to three pounds of beeswax, melted together and boiled for about twenty-five to thirty minutes. These proportions are approximate, and I do not confine myself strictly to them, as a slight variation may be made in them and not change the nature or value of the composition for lubricating.

35 The object of a combination of hemp and

cotton is to secure the greatest elasticity possible—an element very desirable in packing—while it is compact enough for proper tightness. The object in the combination of plumbago, beeswax, and tallow is to secure a mixture that will not dry, but keep a moisture in the packing sufficient to prevent the wasting of the plumbago, which would otherwise occur; also, to keep the lubricating mixture in the most suitable shape for spinning into the cotton and hemp fiber.

50 Engineers and users of steam engines and pumps know from experience the value of packing which is elastic and at the same time possessing lubricating qualities, and in this combination will be found the elements so much desired, viz: durability, elasticity, lubrication, convenience in shape, economy, and excellence in mechanical finish.

55 I am aware that hemp and cotton have been combined in packing, but never heretofore as in this invention. Plumbago has also been used, but never dusted into the fabric when being spun. I therefore do not claim these materials, broadly; but

What I do claim is—

60 The method of making self-lubricating packing for steam and other engines by spinning together equal quantities of hemp and cotton fiber into strands, having pulverized plumbago dusted into the fiber while being spun into strands, and which strands are afterward saturated in a hot mixture of beeswax and tallow, substantially as and for the purpose described.

65 ROBT. MORRISON.

Witnesses:

ED. A. PUSTER,  
A. H. BRUER.